

July 25, 1972

KEISUKE SHIBA ET AL

3,679,428

SPECTRALLY SENSITIZED PHOTOGRAPHIC EMULSIONS

Filed July 23, 1970



INVENTORS

KEISUKE SHIBA, MOTOHIKO TSUBOTA  
AKIRA SATO, TADASHI IKEDA  
AKIRA OGAWA

BY

*Sughrue, Rothwell, Mion  
Zurin & Macpeak*  
ATTORNEYS

1

3,679,428  
SPECTRALLY SENSITIZED PHOTOGRAPHIC  
EMULSIONS

Keisuke Shiba, Motohiko Tsubota, Akira Sato, Tadashi Ikeda, and Akira Ogawa, Kanagawa, Japan, assignors to Fuji Photo Film Co., Ltd., Kanagawa, Japan

Filed July 23, 1970, Ser. No. 57,607  
Claims priority, application Japan, July 23, 1969,  
44/58,180

Int. Cl. G03c 1/08

U.S. Cl. 96—124

6 Claims

### ABSTRACT OF THE DISCLOSURE

A silver halide light-sensitive photographic emulsion containing at least one sensitizing dye represented by the following Formula I:

(Formula I)



in which R is a hydrogen atom or an alkyl group having from 1 to 4 carbon atoms; R<sub>1</sub> and R<sub>2</sub>, which may be the same or different, each represents an alkyl group, an allyl group and an alkyl group substituted by hydroxy, carboxy, sulfo or mixtures thereof, at least one of R<sub>1</sub> and R<sub>2</sub> being a substituted alkyl group; Z<sub>1</sub> is a non-metallic atomic group necessary to complete a heterocyclic nucleus of the naphthothiazole, naphthoselenazole or naphthoxazole series; Z<sub>2</sub> is a non-metallic group necessary to complete a nucleus of the naphthoselenazole, naphthoxazole, naphthoimidazole or benzimidazole series; X<sub>1</sub><sup>-</sup> is an acid anion and n is 1 or 2, and at least one sensitizing dye represented by the following Formula II:

(Formula II)



in which R<sub>5</sub> is an alkyl group having from 1 to 4 carbon atoms; R<sub>3</sub> and R<sub>4</sub>, which may be the same or different, each represents an alkyl group, an allyl group and an alkyl group substituted by hydroxy, alkoxy, carboxy, sulfo or mixtures thereof; Z<sub>3</sub> and Z<sub>4</sub>, which may be the same or different, each represents a non-metallic atomic group necessary to complete a benzothiazole or a benzoselenazole nucleus, which may be substituted by halogen, phenyl, alkoxyphenyl, hydroxyphenyl, carboxyphenyl, an alkyl having from 1 to 4 carbon atoms, hydroxyl, alkoxy, carboxyl, carboxylic acid ester, carbamoyl or alkyl carbamoyl groups; X<sub>2</sub> is an acid anion and m is 1 or 2.

### BACKGROUND OF THE INVENTION

#### Field of the invention

This invention relates to a spectrally sensitized silver halide photographic emulsion and more particularly, it is concerned with a high sensitivity silver halide photographic emulsion which is supersensitized, by the use of a combination of at least two sensitizing dyes over the absorption light wavelength region of each of the sensitizing dyes.

#### Description of the prior art

Ordinarily, conventional photographic light-sensitive materials should be sensitized with a suitable spectral

2

sensitivity over the whole visible wavelength region. As a technique for making such a light-sensitive material, it is well known to add a sensitizing dye to a silver halide photographic emulsion to thus expand its sensitive wavelength region to longer wavelength regions. This phenomenon is termed spectral sensitization.

The spectral sensitization over the visible region is required for light-sensitive materials for photography in general, but having a high spectral sensitivity up to very long wavelengths is not always preferred from the viewpoint of tone reproduction. Two or more sensitizing dyes are generally used in combination in order to obtain the most suitable distribution of spectral sensitivity. However, the spectral sensitivity obtained in the case of using two or more sensitizing dyes in combination to regulate the spectral sensitivity distribution is often lower than in the case of using each of them individually.

The spectral sensitizing action is affected not only by the chemical structure of the sensitizing dye but also by the properties of the silver halide emulsion employed, for example, the crystal habit of the silver halide fine crystals, the particle size, the halogen composition, the hydrogen ion concentration and the silver ion concentration. Furthermore, additives present in the emulsion, such as, for example, inhibitors, stabilizers, sensitizers, hardeners, binders, precipitators, plasticizers, color formers and photographic dyes, have many influences thereupon, many of them acting so as to weaken the special sensitizing action.

In the special case, however, the spectral sensitizing action obtained by adding one sensitizing dye is super-additively strengthened by also adding therewith another sensitizing dye or organic compound, in particular, an aromatic compound. The action of this type is known as supersensitization. The use of a cyanine dye alone scarcely gives a maximum sensitivity over relatively long wavelengths, such as 625 mm. to 640 mm.

It is therefore an object of the present invention to find the spectral sensitization capable of raising the spectral sensitivity of a photographic light-sensitive material, in particular, to a wavelength region of 625 to 640 mm.

It is another object of the present invention to provide a spectral sensitization technique whereby a stable spectral sensitivity and spectral sensitivity distribution are given immediately after addition of two or more sensitizing dyes to a silver halide emulsion. Such a technique is very important for improving the productivity in making photographic light-sensitive materials.

Other objects and advantages will be apparent from the following description.

#### SUMMARY OF THE INVENTION

The present inventors have found that the above-mentioned objects can favorably be accomplished by providing a silver halide light-sensitive photographic emulsion having incorporated therein at least one sensitizing dye represented by the following general Formula I and at least one cyanine dye represented by the following general Formula II:

(General Formula I)



wherein R represents a hydrogen atom or a lower alkyl group, such as methyl or ethyl; R<sub>1</sub> and R<sub>2</sub>, which may be the same or different, are selected from groups of the alkyl series, such as alkyl groups (e.g., methyl, ethyl and propyl), allyl groups and substituted alkyl groups (e.g.,

2-hydroxyethyl, carboxymethyl, 3-carboxypropyl, 3-sulfo-propyl, 4-sulfobutyl, 3-sulfoisobutyl, and 2-hydroxy-3-sulfopropyl groups), at least one of  $R_1$  and  $R_2$  being a substituted alkyl group of the type indicated;  $Z_1$  represents a non-metallic atomic group necessary to complete a heterocyclic nucleus of the naphthothiazole series (e.g.,  $\alpha$ -naphthothiazole,  $\beta$ -naphthothiazole, 5-methoxy- $\beta$ -naphthothiazole, 5-ethoxy- $\beta$ -naphthothiazole, 8-methoxy- $\alpha$ -naphthothiazole, 7 - methoxy -  $\alpha$  - naphthothiazole), the naphthoselenazole series (e.g.,  $\alpha$ -naphthoselenazole or  $\beta$ -naphthoselenazole), or the naphthoxazole series (e.g.,  $\alpha$ -naphthoxazole or  $\beta$ -naphthoselenazole);  $Z_2$  represents a non-metallic atomic group necessary to complete a heterocyclic nucleus of the naphthoxazole series (e.g.,  $\alpha$ -naphthoxazole or  $\beta$ -naphthoxazole), the naphthoimidazole series (e.g.,  $\alpha$ -naphthoimidazole or  $\beta$ -naphthoimidazole) or the benzimidazole series (e.g., 3-ethyl-5,6-dichlorobenzimidazole, 3 - ethyl-5-ethylsulfonyl-6-trifluoromethylbenzimidazole, 3 - hydroxyethyl - 5 - cyano-6-bromo-benzimidazole, 3-acetoxypropyl - 5 - morpholinosulfonyl-benzimidazole, 3-propyl - 6 - ethylcarbamoyl-benzimidazole);  $X_1^-$  represents an acid anion usually employed in the field of sensitizing dyes, such as a halogen ion, perchlorate, thiocyanate, benzenesulfonate, p-toluene sulfonate, ethylsulfate, a methylsulfate ion, and the like and  $n$  represents 1 or 2.

(General Formula II)



wherein  $R_5$  represents a lower alkyl group, such as ethyl or butyl;  $R_3$  and  $R_4$ , which may be the same or different, each represents groups of the alkyl series, such as alkyl groups (e.g., methyl, ethyl and butyl), allyl groups and substituted alkyl groups (e.g., 2-hydroxyethyl, 2-methoxyethyl, carboxymethyl, 3-carboxypropyl, 4-carboxybutyl, 3-sulfopropyl, 4-sulfobutyl, 3-sulfoisobutyl, 2-(3-sulfopropoxy)ethyl and 2-hydroxy-3-sulfopropyl);  $Z_3$  and  $Z_4$ , which may be the same or different, each represents a non-metallic atomic group necessary to complete a benzothiazole or a benzoselenazole nucleus which may be substituted by a group capable of promoting the formation of the J-aggregate, for example, a halogen atom such as chlorine or bromine, a phenyl group, a substituted phenyl group such as p-methoxy phenyl, o-hydroxyphenyl, p-carboxyphenyl, a lower alkyl group (such as methyl or ethyl), a hydroxyl group, an alkoxy group such as methoxy, a carboxyl group, a carboxylic acid ester (such as carboxymethyl or carboxyethyl), a carbamoyl group or an alkyl carbamoyl group;  $X_2^-$  represents an acid anion usually employed in the field of sensitizing dyes, such as halogen, perchlorate, benzenesulfonate, thiocyanate, p-toluene sulfonate, methylsulfate, ethylsulfate and the like, and  $m$  represents 1 or 2.

#### BRIEF DESCRIPTION OF THE DRAWINGS

The figure represents spectrograms of samples containing a dye of Formula I, a dye of Formula II and a combination thereof, respectively.

## **DETAILED DESCRIPTION OF THE PREFERRED EMBODIMENTS**

The most important features of the present invention are that, in the sensitizing dye represented by Formula I, the nitrogen atom in the cyanine dye nuclei consisting of the naphthothiazole, naphthoselenazole, naphthoxazole or naphthoimidazole nucleus is substituted by at least one substituted alkyl group as described above, and that the cyanine dye represented by Formula II is liable to form a relatively strong J-aggregate. The supersensitizing action over the whole wavelength region which the dyes absorb is obtained and the spectral sensitivity distribution is regu-

lated relatively optional by the use of, in combination, the sensitizing dye characterized by the chemical structure of Formula I and the cyanine dye represented by Formula II in suitable amounts. In particular, the spectral sensitivity 5 within a wavelength region of 625 mm. to 640 mm. can be raised. A further feature of the present invention consists in the advantage that the supersensitization given by the sensitizing dye of Formula I serves to markedly improve the stability and reproducibility of the spectral sensitivity 10 obtained.

The sensitizing dyes of the present invention are dissolved in an aqueous solution or in a water-soluble organic solvent such as methanol, ethanol, acetone, methyl Cello-solve or pyridine and then added to a silver halide emulsion separately or as a mixture thereof. Stirring by ultrasonic waves may be applied during the dissolving of the sensitizing dyes. The amount of addition, order of addition and addition procedure may be varied with the production process of the light-sensitive material. The amount of addition of the sensitizing dyes is preferably from  $1 \times 10^{-6}$  mole to  $5 \times 10^{-4}$  mole per mole of silver halide, the molar ratio of the sensitizing dye represented by Formula I to the cyanine dye represented by Formula II being within the range 10 to 100:1, preferably 4:1.

25 As the silver halide emulsion of the present invention, silver iodobromide, iodochloride or chlorobromide is preferably used. To such emulsions may be applied conventional chemical sensitizing methods as well as fog inhibitors, stabilizers, sensitizers, surfactants, hardeners, 30 plasticizers and photographic dyes. The resulting emulsion is coated onto a suitable support, for example, a cellulose derivative film, a polyethylene terephthalate film, a polycarbonate film, baryta paper, resin coated paper, synthetic paper, resin laminated paper or a glass sheet.

35 Examples of the sensitizing dyes according to the present invention are given below, these compounds being merely illustrative and not limiting in nature.

### Sensitizing dyes represented by general Formula I:



### Cyanine dyes represented by general Formula II:





The sensitizing dyes represented by Formulae I and II may be synthesized in any known manner. For example, dyes IA, IB, IIA, IIB, IIC, IID and IIE can be readily synthesized by the methods disclosed in U.S. Pat. No. 2,503,776, German Pats. Nos. 929,080 and 1,072,765 and

Sensitizing dyes represented by Formulae I and II were separately dissolved in methanol to give a predetermined concentration (shown in Table I). A predetermined amount (shown in Table I) of each of the sensitizing dye solutions was added to the emulsion with agitation. After 10 minute, 7 ml. of each emulsion was applied to a glass sheet of cabinet size and dried to obtain a sample.

One of the samples, which was then cut, was subjected to optical wedge exposure through a K-12 yellow filter (trademark) and a K-7 red filter (trademark) made by Fuji Photo Film Co., Ltd., using an actinometer having a light source whose color temperature is converted into 5400° K. by applying a David-Gibson conversion filter to a light source of a color temperature of 2666° K. The other sample was exposed to obtain a spectrogram by the use of a spectrophotograph of the diffraction grating type (GR-2 [trademark], made by Narumi Co.).

The first sample was then developed with a developer having the following composition at 20° C. for 10 minutes and then subjected to stopping, fixing and water washing to obtain a strip whose density was measured using an S-type densitometer (trademark) made by Fuji Photo Film Co., Ltd., to thus obtain the yellow filter sensitivity (Sy), red filter sensitivity (Sr) and predetermined maximum sensitivity wavelength (S<sub>max</sub>), respectively. The standard point of optical density to determine the sensitivity is at a point of (fog + 0.20).

Composition of developer:

|                          |     |     |
|--------------------------|-----|-----|
| Water (50° C.)           | ml. | 750 |
| Metol                    | g.  | 2   |
| Anhydrous sodium sulfite | g.  | 100 |
| Hydroquinone             | g.  | 5   |
| Borax                    | g.  | 2   |

Water to make 1000 ml.

TABLE I

| Test number | Dye | Amount of methanol used, ml. (mol conc.) | Dye  | Amount of methanol used, ml. (mol conc.) |     |      | Relative sensitivity | S <sub>max</sub> (mm.) |     |
|-------------|-----|------------------------------------------|------|------------------------------------------|-----|------|----------------------|------------------------|-----|
|             |     |                                          |      | Sy                                       | Sr  | Fog  |                      |                        |     |
| 1           | IA  | 10 (5×10 <sup>-4</sup> )                 |      | 191                                      | 85  | 0.12 | 620                  |                        |     |
|             |     | 20                                       |      | 100                                      | 100 | 0.15 | 620                  |                        |     |
|             |     | 40                                       |      | 85                                       | 90  | 0.16 | 620                  |                        |     |
|             |     |                                          | IIA  | 5 (1×10 <sup>-3</sup> )                  | 56  | 63   | 0.12                 | 645                    |     |
| 2           |     |                                          |      | 10                                       | 113 | 113  | 0.12                 | 650                    |     |
|             |     |                                          |      | 20                                       | 113 | 115  | 0.14                 | 650                    |     |
|             |     |                                          |      | 5 (1×10 <sup>-3</sup> )                  | 180 | 160  | 0.12                 | 630                    |     |
|             |     |                                          |      | 10                                       | 180 | 160  | 0.12                 | 640                    |     |
| 3           | IA  | 20 (5×10 <sup>-4</sup> )                 |      | 20                                       | 180 | 160  | 0.14                 | 645                    |     |
|             |     | 20                                       | IIA  | 5 (1×10 <sup>-3</sup> )                  | 130 | 130  | 0.12                 | 630                    |     |
|             |     | 20 (5×10 <sup>-4</sup> )                 |      | 10                                       | 167 | 145  | 0.13                 | 630                    |     |
|             |     | 20                                       |      | 20                                       | 183 | 150  | 0.14                 | 640                    |     |
| 4           | IA  | 20                                       | IIIB | 10 (1×10 <sup>-3</sup> )                 | 25  | 90   | 0.10                 | 645                    |     |
|             |     | 20                                       |      | 20                                       | 125 | 120  | 0.10                 | 645                    |     |
|             |     | 20                                       |      | 40                                       | 135 | 130  | 0.12                 | 660                    |     |
|             |     |                                          |      | 90                                       | 90  | 0.11 | 624                  |                        |     |
| 5           | IIB | 10 (5×10 <sup>-4</sup> )                 |      | 105                                      | 100 | 0.12 | 624                  |                        |     |
|             |     | 20                                       |      | 110                                      | 100 | 0.13 | 624                  |                        |     |
|             |     | 40                                       |      | 5 (1×10 <sup>-3</sup> )                  | 60  | 70   | 0.11                 | 656                    |     |
|             |     |                                          |      | 10                                       | 110 | 110  | 0.12                 | 656                    |     |
| 6           | IB  |                                          |      | 20                                       | 120 | 116  | 0.12                 | 660                    |     |
|             |     |                                          |      | 5 (1×10 <sup>-3</sup> )                  | 170 | 160  | 0.12                 | 630                    |     |
|             |     |                                          |      | 10                                       | 175 | 175  | 0.14                 | 650                    |     |
|             |     |                                          |      | 20                                       | 185 | 175  | 0.14                 | 650                    |     |
| 7           | IID |                                          |      | 5 (5×10 <sup>-4</sup> )                  | 110 | 105  | 0.12                 | 625                    |     |
|             |     |                                          |      | 10                                       | 125 | 118  | 0.12                 | 630                    |     |
|             |     |                                          |      | 20                                       | 130 | 128  | 0.13                 | 650                    |     |
|             |     |                                          |      | 5 (5×10 <sup>-4</sup> )                  | 61  | 93   | 0.09                 | 630                    |     |
| 8           | IB  | 20 (5×10 <sup>-4</sup> )                 |      | 10                                       | 80  | 100  | 0.12                 | 630                    |     |
|             |     | 20                                       |      | 20                                       | 74  | 79   | 0.14                 | 630                    |     |
|             |     | 20 (5×10 <sup>-4</sup> )                 |      | 200                                      | 132 | 132  | 0.09                 | 618                    |     |
|             |     | 20                                       |      | 226                                      | 132 | 132  | 0.14                 | 618                    |     |
| 9           | IIC | 20                                       |      | 146                                      | 71  | 0.14 | 618                  |                        |     |
|             |     | 40                                       |      | 226                                      | 150 | 0.16 | 620                  |                        |     |
|             |     | 20                                       |      | 10                                       | 250 | 155  | 0.18                 | 620                    |     |
|             |     | 20                                       |      | 20                                       | 300 | 180  | 0.25                 | 620                    |     |
| 10          | IIC | 20 (5×10 <sup>-4</sup> )                 |      | 5 (5×10 <sup>-4</sup> )                  | 50  | 60   | 0.08                 | 623                    |     |
|             |     | 20                                       |      | 10                                       | 50  | 70   | 0.08                 | 623                    |     |
|             |     | 20                                       |      | 20                                       | 50  | 75   | 0.09                 | 623                    |     |
|             |     |                                          |      |                                          |     |      |                      |                        |     |
| 11          | IC  | 10 (1×10 <sup>-3</sup> )                 |      |                                          |     |      |                      |                        |     |
|             |     | 20                                       |      |                                          |     |      |                      |                        |     |
|             |     | 40                                       |      |                                          |     |      |                      |                        |     |
|             |     |                                          |      |                                          |     |      |                      |                        |     |
| 12          | IC  | 20 (1×10 <sup>-3</sup> )                 |      | 5 (5×10 <sup>-4</sup> )                  | 10  | 250  | 155                  | 0.18                   | 620 |
|             |     | 20                                       |      | 20                                       | 300 | 180  | 0.25                 | 620                    |     |
|             |     | 20                                       |      | 5 (5×10 <sup>-4</sup> )                  | 50  | 60   | 0.08                 | 623                    |     |
|             |     | 20                                       |      | 10                                       | 50  | 70   | 0.08                 | 623                    |     |
| 13          | IIE |                                          |      | 20                                       | 50  | 75   | 0.09                 | 623                    |     |
|             |     |                                          |      |                                          |     |      |                      |                        |     |
|             |     |                                          |      |                                          |     |      |                      |                        |     |
|             |     |                                          |      |                                          |     |      |                      |                        |     |

dye IC can be readily synthesized by the methods disclosed in British Pats. Nos. 776,050 and 979,251.

EXAMPLES

500 g. of a silver iodobromide photographic emulsion (iodine content: 4.0 mole percent), prepared in a conventional manner and chemically aged, was placed in a beaker and rendered molten in a thermostat at 40° C. 75

The resulting spectrograms are shown in FIG. 1, where in curve 1 is a spectrogram of the sample obtained by adding 20 ml. of sensitizing dye (IA) of No. 1 in Table I; curve 2 is a spectrogram of the sample obtained by adding 10 ml. of sensitizing dye (IIA) of No. 2 in Table I; and curve 3 is a spectrogram of the sample obtained by adding a mixture of 20 ml. of dye (IA) and 10 ml. of dye (IIA) according to the present invention.

What is claimed is:

1. A silver halide light-sensitive photographic emulsion containing at least one sensitizing dye represented by the following Formula I:

(Formula I)



in which R is a hydrogen atom or an alkyl group having from 1 to 4 carbon atoms; R<sub>1</sub> and R<sub>2</sub>, which may be the same or different, each represents an alkyl group, an allyl group and an alkyl group substituted by hydroxy, carboxy, sulfo or mixtures thereof, at least one of R<sub>1</sub> and R<sub>2</sub> being a substituted alkyl group; Z<sub>1</sub> is a non-metallic atomic group necessary to complete a heterocyclic nucleus of the naphthothiazole, naphthoselenazole or naphthoxazole series; Z<sub>2</sub> is a non-metallic group necessary to complete a nucleus of the naphthoselenazole, naphthoxazole, naphtho-imidazole or benzimidazole series; X<sub>1</sub><sup>-</sup> is an acid anion and n is 1 or 2, and at least one sensitizing dye represented by the following Formula II:

(Formula II)



in which R<sub>5</sub> is an alkyl group having from 1 to 4 carbon atoms; R<sub>3</sub> and R<sub>4</sub>, each represents a member selected from the group consisting of sulfoalkyl and hydroxyalkyl groups; Z<sub>3</sub> and Z<sub>4</sub>, which may be the same or different, each represents a non-metallic atomic group necessary to complete a benzothiazole or a benzoselenazole nucleus, which may be substituted by halogen, phenyl, alkoxy-phenyl, hydroxyphenyl, carboxyphenyl, an alkyl having from 1 to 4 carbon atoms, hydroxyl, alkoxy, carboxyl, carboxylic acid ester, carbamoyl or alkyl carbamoyl groups; X<sub>2</sub> is an acid anion and m is 1 or 2.

2. A silver halide light-sensitive photographic emulsion as in claim 1, wherein said sensitizing dyes represented by Formulae I and II are, respectively,



and



3. The silver halide light-sensitive photographic emulsion as in claim 1, wherein said sensitizing dyes represented by Formulae I and II are, respectively,



4. The silver halide light-sensitive photographic emulsion of claim 1, wherein said dyes are present in an amount of from  $1 \times 10^{-6}$  to  $5 \times 10^{-4}$  mole per mole of silver halide in said emulsion and wherein the molar ratio of said dye of Formula I to said dye of Formula II varies from 10:1 to 100:1.

5. The photographic light-sensitive element comprising a support having thereon at least one layer containing the silver halide light-sensitive photographic emulsion of claim 1.

6. A silver halide light-sensitive photographic emulsion containing at least one sensitizing dye represented by the following Formula I:

(Formula I)



in which R is a hydrogen atom or an alkyl group having from 1 to 4 carbon atoms; R<sub>1</sub> and R<sub>2</sub>, which may be the same or different, each represents an alkyl group, an allyl group and an alkyl group substituted by hydroxy, carboxy, sulfo or mixtures thereof, at least one of R<sub>1</sub> and R<sub>2</sub> being a substituted alkyl group; Z<sub>1</sub> is a non-metallic atomic group necessary to complete a heterocyclic nucleus of the naphthothiazole, or naphthoselenazole series; Z<sub>2</sub> is a non-metallic group necessary to complete a nucleus of the naphthoselenazole, naphtho-imidazole or benzimidazole series; X<sub>1</sub><sup>-</sup> is an acid anion and n is 1 or 2, and at least one sensitizing dye represented by the following Formula II:

(Formula II)



in which R<sub>5</sub> is an alkyl group having from 1 to 4 carbon atoms; R<sub>3</sub> and R<sub>4</sub>, each represents a member selected from the group consisting of sulfo alkyl and hydroxyalkyl groups; Z<sub>3</sub> and Z<sub>4</sub>, which may be the same or different, each represents a non-metallic atomic group necessary to complete a benzothiazole or a benzoselenazole nucleus, which may be substituted by halogen, phenyl, alkoxy-phenyl, hydroxyphenyl, carboxyphenyl, an alkyl having from 1 to 4 carbon atoms, hydroxyl, alkoxy, carboxyl, carboxylic acid ester, carbamoyl or alkyl carbamoyl groups; X<sub>2</sub> is an acid anion and m is 1 or 2.

#### References Cited

#### UNITED STATES PATENTS

|           |        |                 |        |
|-----------|--------|-----------------|--------|
| 3,463,640 | 8/1969 | Ficken et al.   | 96-124 |
| 3,459,553 | 8/1969 | Walworth        | 96-124 |
| 3,338,714 | 8/1967 | Ficken et al.   | 96-124 |
| 3,527,641 | 9/1970 | Nakazawa et al. | 96-124 |
| 3,573,920 | 4/1971 | Hiller          | 96-124 |

#### OTHER REFERENCES

Ser. No. 57,766, filing date July 23, 1970, by Nakazawa et al.

70 NORMAN G. TORCHIN, Primary Examiner

E. C. KIMLIN, Assistant Examiner

U.S. CL. X.R.